

March 12, 1940.

H. MASUMOTO ET AL

2,193,768

MAGNETIC ALLOYS

Filed Sept. 14, 1937



INVENTORS  
HAKARU MASUMOTO  
BY TATSUJI YAMAMOTO

*Hammond & Littell*  
ATTORNEYS

## UNITED STATES PATENT OFFICE

2,193,768

## MAGNETIC ALLOYS

Hakaru Masumoto and Tatsuji Yamamoto,  
Sendai, Japan, assignors to The Kinzoku Zairyo  
Kenkyusho, Sendai, Japan

Application September 14, 1937, Serial No. 163,776  
In Japan February 6, 1932

5 Claims. (Cl. 75—124)

This invention relates to magnetic alloys having very high permeability and specific resistance and very low hysteresis loss.

Many magnetic alloys are known to the prior art, such as iron-silicon alloys and permalloys, which materials have been used as magnetic cores in various electric machines and apparatus such as transformers, leading coils and the like. The best silicon-iron alloy known up to the time of 10 the present invention has contained about 4% of silicon, the remainder being iron.

Although these heretofore known alloys have been used to quite a large extent, they are not completely suitable for these purposes in several 15 of their properties. Furthermore, a magnetic alloy of iron, silicon, aluminum and optionally also phosphorous is suggested in the prior art, but the proportions of the ingredients used did not provide products of high quality.

20 The principal object of the present invention is to produce alloys for electromagnetic uses which have much higher permeability, greater specific resistance and less hysteresis loss than the alloys heretofore known.

25 As the result of exhaustive experiments, we have discovered that silicon-aluminum-iron alloys can be produced which have superior magnetic properties to those known to the prior art, including the above mentioned alloys. These new alloys may be manufactured at a low cost through very 30 simple operations. An exceedingly valuable alloy constituting one example of the present invention contains 9.5% of silicon and 4.5% of aluminum, the remainder being iron, which alloy possesses a very high initial permeability and other 35 outstanding properties.

We have furthermore discovered that the proportions of these three metals may be varied considerably from the optimum proportions giving 40 the highest initial permeability characteristics, and yet obtain alloys having other highly desirable magnetic properties. For example, most of the alloys producible within the ranges of 3.5 to 12% of silicon, 3 to 12% of aluminum and 81.5 to 91% of iron have an initial permeability 45 in excess of 1500 mu and also other superior magnetic properties. Alloys of good properties are likewise obtained within the broader ranges of 0.5 to 16% or 2 to 13% of silicon, 0.5 or 2 to 16% of aluminum and not more than 90 or 91% of iron, preferably from 80 to 89%. An increase in 50 the percentages of the non-ferrous metals from these minimums leads to better products. For example, the alloys of silicon in the proportion of 6 or 7 to 11%, of the aluminum in the proportion of 4 to 8 or 9%, the remainder (82 to 88%) being of iron are excellent.

In producing the alloys of the present invention, the several metals are mixed together in 55 the proper proportions and melted in any suit-

able apparatus as through the use of an induction furnace. The molten mass may then be cast in an suitable iron mold. Thereafter, it is heat treated by an annealing operation at about 1000° C. for a suitable period, as for several hours, and the mass is then allowed to cool slowly in order to develop the required properties.

The excellent properties of two alloys within the scope of the present invention as compared with a most common prior alloy may be observed 10 from the following table. The alloy A in the table comprises one which is frequently used for transformers and contains about 4% of silicon. The alloy B, constituting an example of an alloy 15 of the present invention, contains 9.5% of silicon, 4.5% of aluminum and 86% of iron. The alloy C, constituting another example of the present invention, contains 9.5% of silicon, 6% of aluminum and 84.5% of iron. The superiority of the 20 alloys of the present invention may be readily observed from the experimental results as here recorded.

|                                                                                                       | Alloy A | Alloy B | Alloy C |
|-------------------------------------------------------------------------------------------------------|---------|---------|---------|
| Initial permeability                                                                                  | 300     | 5,500   | 30,000  |
| Maximum permeability                                                                                  | 7,000   | 80,000  | 120,000 |
| Hysteresis loss (at the maximum magnetic induction of 10,000 gauss in ergs/cm <sup>3</sup> per cycle) | 1,450   | 180     | 90      |
| Specific resistance in micro-ohms/cub. cm                                                             | 50      | 75      | 80      |

The results recorded in the above table show clearly that the alloys of the present invention possess a much greater permeability and specific resistance and have less hysteresis loss than the alloys of the usual iron-silicon composition which have been known up to the present time as the best magnetic material of this nature.

In order to illustrate the superiority of the 40 alloys of the present invention, a drawing is submitted herewith showing diagrams upon which the initial permeabilities (Figure 1) and the maximum permeabilities (Figure 2) of the various alloys within the scope of the present invention are recorded. The diagrams reveal the relative effectiveness of the various proportions of the silicon, aluminum and iron in the alloys with respect to these properties. It should be understood therefore that the drawing is concerned with only two of the superior properties of the present compositions and that other good properties, such as the magnetic induction and the magnetic hysteresis loss, the residual magnetic induction, the coercive force, the magnetic intensity, the specific electric resistance and the average temperature coefficient for electric resistance are not shown. It is believed, however, that the superiority of the alloys of the present invention is readily apparent from the drawing. From Figure 1 of this drawing, it will be noted 50

that alloys of good initial permeability are obtained where the metals are in the proportions described herein. It will also be observed that alloys of rather high permeability are obtained 5 through the use of over 5% and up to 12% of silicon and from 2 to 10% of aluminum, the remainder being iron. When the alloy contains from 6.5 to 10.5% of silicon and from 4 to 8% of aluminum, alloys of high permeability are obtained. As the silicon is increased from 5 or 5.5% 10 to about 9%, and the aluminum to about 6%, the permeability is increased to an extremely high degree.

An initial permeability equal to or in excess of 15 20,000 mu is obtained when the silicon content is from 8.6 to 9.8% and the aluminum content from 5.2 to 7%. This property reaches the highest value of 35,100 mu when the silicon constitutes about 9.62% and the aluminum constitutes 20 5.38%, the maximum permeability of the alloy being 117,500 mu.

As may be observed from Figure 2, the maximum permeability of the alloys of the present invention containing 6.5% of silicon gradually increases as the aluminum content is increased. A maximum permeability of 54,000 mu is reached 25 when the silicon is at about 5.5% and the aluminum about 3%, the addition of further aluminum causing this value to decrease. When the silicon content is increased and constitutes from 30 7 to 11% and the aluminum content is from 4 to 8%, the remainder being iron, an extremely high maximum permeability is obtained, the value reaching 162,000 mu when the alloy contains about 9.66% of silicon and 6.21% of aluminum.

Magnetic materials suitable for electrical machines and devices require a high permeability and small hysteresis loss and also a high electric specific resistance, the latter quality serving the purpose of reducing the change of permeability due to the variation of the field strength and also to obtain a small eddy current loss. For some purposes the magnetic materials should possess 40 a greater electrical resistance and a smaller variation of permeability at the expense of some reduction of permeability. For these reasons, the alloys of the present invention may be modified by the addition of other metals or metalloids which may be added in a quantity amounting to 45 less than 40% as to their total sum. Metals of the nature of nickel, cobalt, chromium, tungsten, molybdenum, manganese, vanadium, titanium, tin and zinc may be added in a quantity not in excess of about 10%. The metals magnesium, 50 antimony, tantalum and beryllium may be added in an amount which should not exceed about 5%. The metals boron, copper and phosphorous may be incorporated in the alloy in quantities not exceeding about 2%. Arsenic, sulfur and zirconium may be used in small amounts. With 55 reference to all of these metals, the quantity used must be insufficient to destroy the herein described magnetic properties of the resulting alloy. The addition of most any of these substances even in small amounts, will result in an increase in the electric resistance or in less change of permeability for different intensities of the magnetic field. The addition of any other 60 element besides the above mentioned metals to the iron-silicon-aluminum alloys of the present invention will generally increase the electric resistance without excessively impeding their magnetic properties. Up to 7% of manganese, tin or 65 vanadium, or up to 2% of antimony, or up to 5%

of chromium may be used to produce alloys of special magnetic properties of particular interest in the arts.

In order to illustrate the effect of the addition of a metal, the following table is recorded from 5 experimental results:

| Si,<br>percent | Al,<br>percent | Added element— |                | Initial per-<br>meability,<br>mu | Specific re-<br>sistance<br>micro-ohms/<br>cu. cm. | 10 |
|----------------|----------------|----------------|----------------|----------------------------------|----------------------------------------------------|----|
|                |                | Fe,<br>percent | Mn,<br>percent |                                  |                                                    |    |
| 9.5            | 6.0            | 84.5           | —              | 30,000                           | 80                                                 | 15 |
| 9.1            | 5.8            | 81.2           | 3.9            | 30,000                           | 120                                                |    |
| 8.6            | 6.4            | 75.9           | 9.1            | 10,000                           | 180                                                |    |

It will be observed from the above table that the addition of manganese to typical alloys of the present invention increases the specific electric resistance without lowering the initial permeability to a prohibitive degree.

From the experimental results hereinbefore set out, it is evident that the alloys of the present invention are exceedingly well adapted for use as magnetic materials for transformers and other electric machines and devices. They are particularly suitable either in the form of solid cores or dust cores of loading coils used in telephone systems.

The superior magnetic properties of the alloys of the present invention are attributable mainly to the discovery of the most effective proportions of silicon and aluminum content of the silicon-aluminum-iron alloys. For example, alloys possessing an initial permeability of a minimum of 2,000 mu may be produced by formation of an alloy containing from 4 to 11% silicon and from 3.5 to 11% aluminum.

The iron employed may satisfactorily be that which is known as electrolytic iron which is substantially free of other metals and of non-metals including carbon.

The alloys of the present invention may be cast or molded into the form of a sheet or they may be crushed into particles or powders in which form they are adapted for use in the production 45 of dust cores of loading coils.

This application is a continuation-in-part of the applicants' copending application Serial No. 652,101, filed January 16, 1933.

It should be understood that the present invention is not limited to the specific proportions and treatment herein described but that it extends to all equivalents coming within the scope of the appended claims.

We claim:

1. A substantially carbon-free ternary magnetic alloy adapted for use in magnetic parts of electric machines and devices composed of over 5% up to 12% of silicon, 2 to 10% of aluminum and the remainder of iron.

2. A magnetic alloy for electromagnetic purposes composed of 8.6 to 9.8% of silicon, 5.2 to 7% of aluminum and the remainder iron.

3. A magnetic alloy for electromagnetic uses composed of 9.5% of silicon, 4.5% of aluminum and 86% of iron.

4. A magnetic alloy for electromagnetic uses composed of 9.5% of silicon, 6.0% of aluminum and 84.5% of iron.

5. An electromagnetic alloy composed of 9.62% of silicon, 5.38% of aluminum and the remainder iron.

HAKARU MASUMOTO.  
TATSUJI YAMAMOTO. 75